

# UNITED STATES PATENT OFFICE.

JOHN W. RADU, OF NEW YORK, N. Y., ASSIGNOR TO WESTERN ELECTRIC COMPANY,  
INCORPORATED, OF NEW YORK, N. Y., A CORPORATION OF NEW YORK.

## LEADING-IN CONDUCTOR.

1,426,771.

Specification of Letters Patent. Patented Aug. 22, 1922.

No Drawing.

Application filed January 16, 1920. Serial No. 351,977.

To all whom it may concern:

Be it known that I, JOHN WILLIAM RADU, a citizen of the United States, residing at New York, in the county of New York and 5 State of New York, have invented certain new and useful Improvements in Leading-In Conductors, of which the following is a full, clear, concise, and exact description.

This invention relates to improvements in 10 leading-in conductors for mercury arc rectifiers, vacuum tubes, incandescent lamps and the like.

Platinum and platinum alloys have been used extensively in the past for leading-in 15 wires in such devices on account of two important properties which such substances have. In the first place, platinum and its alloys with the nobler metals are not oxidized upon being exposed to the atmosphere, even 20 at high temperatures. Thus when wire composed of such materials is heated preparatory to being sealed in glass, no oxide coating will form on its surface to prevent a satisfactory tight seal from being made. In 25 the second place, such a wire will possess the same or approximately the same coefficient of expansion as that of the glass employed. This fact will prevent any disruption of the seal when the glass becomes heated during 30 use. While no material has been found which will act in the same manner as platinum in this connection, it is possible to so treat materials such as the baser metals, which have not these properties per se, that 35 they may be readily utilized for the above-named purpose.

An object of the invention is to so treat wire composed of one or more of the baser metals that it may be used as a leading-in 40 wire.

It is well-known that the two salts, sodium borate and sodium meta-phosphate, possess the property of uniting chemically with metallic oxides under the influence of heat to 45 form new compounds. In fact both of these salts have had wide use as reagents in qualitative analysis of the metals, a different color being given to the molten salt by the different oxides so treated. These salts also have 50 been used as fluxes for sealing wire into glass. In such a case the wire is dipped into either the moistened salt or its solution, heated for a moment and then forced into the heated glass. It has been observed, however, 55 that when the sodium meta-phosphate

salt is employed for sealing wire into glass a seal, which is similar to that obtained with platinum and the like, is readily secured. Upon examination this has been found to be due to a chemical union between the superimposed phosphate salt and the surface skin of the wire. The superiority of the phosphate salt, therefore, is due to this superficial welding of the flux coating to the metal itself. 60

In carrying out this invention a concentrated aqueous solution of microcosmic salt  $\text{NaNH}_2\text{HPO}_4 \cdot 4\text{H}_2\text{O}$  is prepared. The exact percentage composition of this bath will be governed by the thickness of the final coating desired. The wire to be coated, such as copper, iron, iron-nickel, etc., is then passed slowly through the bath and upon emerging therefrom is covered with a thin film of this solution. It then passes through warm dry 75 air, where the water of solution and of crystallization is entirely driven off and a continuous coating of the anhydrous salt remains. The wire then enters a chamber which is kept at a much higher temperature, 80 i. e., one which is capable of causing a gradual fusion of the salt to take place. As this occurs, water of constitution and ammonia are expelled, leaving sodium meta-phosphate  $\text{NaPO}_4$ . As this compound is formed, it at 85 once reacts with the metallic oxide which is present on the surface of the wire and forms a compound having a complex anion. Thus if the wire be made of copper, the compound formed would be  $\text{NaCuPO}_4$ . At this same 90 temperature, however, the salt becomes welded to the surface of the wire. No attempt will be made to assign any particular formula to the compound thus produced since it appears rather to be in the nature of a solution of the surface skin of the wire in the flux coating. 95

After the above treatment, the wire is slowly cooled and then reeled. The reels may then be stored until desired for use 100 without danger of subsequent cracking off of the flux coating. Wire thus prepared, is admirably suited for leading-in wires, inasmuch as the operator does not have to add the flux at the time the seal is made. There 105 is also the added advantage that the amount of flux required which depends somewhat upon the chemical composition of the glass employed and which may be predetermined, is present in the right proportions and no 110

extraordinary skill in this connection on the part of the operator is necessary.

While sodium meta-phosphate has been referred to herein, other phosphates which 5 have the properties of fusing and uniting with the oxide and surface skin of the metal, may be used.

What is claimed is:

1. A leading-in conductor comprising a 10 base metal and having a baked-on coating of a phosphate.
2. A leading-in conductor of a base metal or metals comprising a moisture-free coating of a phosphate.
- 15 3. A leading-in conductor composed of copper, having superimposed thereon a baked-on coating of sodium meta-phosphate.
4. A leading-in conductor of a base metal or metals comprising a baked-on flux coating 20 which is welded to said conductor.

5. A leading-in conductor of a base metal or metals comprising a baked-on flux coating which is chemically united to said conductor.

6. A leading-in conductor having a baked-on coating of phosphate. 25

7. A leading-in conductor composed of copper, having superimposed thereon a baked-on coating of a phosphate.

8. A leading-in conductor of a base metal or metals comprising a baked-on flux coating 30 of a phosphate which is welded to said conductor.

9. A leading-in conductor of a base metal or metals comprising a baked-on flux coating 35 of a phosphate which is chemically united to said conductor.

In witness whereof, I hereunto subscribe my name this 14th day of January, A. D. 1920.

JOHN W. RADU.